

1

2,955,944

## ELECTROLESS NICKEL PLATING BATH CONTROL

Robert A. Spaulding, Huntington Woods, Mich., assignor to General Motors Corporation, Detroit, Mich., a corporation of Delaware

No Drawing. Filed July 3, 1953, Ser. No. 366,069

7 Claims. (Cl. 106—1)

This invention relates to improvements in the deposition of nickel from chemical reduction plating solutions and more particularly to an improved plating bath, its control and maintenance.

It is known that nickel can be deposited on certain types of metals by immersion of the metal in an aqueous solution of a nickel salt and a reducing agent such as sodium hypophosphite or potassium hypophosphite. There are two general types of such plating solutions, namely, alkaline and acid, of which the acid solution is better adapted for commercial type plating operations. The plating is usually conducted at a temperature of about 90° C. or higher in the presence of certain catalytic metals which initiate the oxidation-reduction plating reaction.

The products of the plating reaction are metallic nickel, which is deposited on the metal article immersed in the solution, sodium dihydrogen phosphite and/or phosphate, and hydrochloric acid. Since optimum nickel deposits are obtained at a pH within the range of about 4 to 6, it will be seen that continued operation of this type plating bath results in an undesirable lowering of the pH by the accumulation of hydrochloric acid.

Accordingly, for continuous or extended plating operations it is necessary, in addition to replenishing the nickel and reducing agent as they are used up, to regulate the bath pH by additions of an alkali. In the past, this has been accomplished by additions of a water soluble nickel salt such as nickel chloride, an alkali such as sodium hydroxide, and a reducing agent, generally sodium hypophosphite.

However, prior reduction plating bath replenishment techniques, in addition to requiring extremely accurate pH determinations, involve certain difficulties because of the by-products formed during the interreaction of the added ingredients. For example, in a typical chemical reduction plating bath, utilizing nickel chloride, which has been in use for some time there are quantities of hydrochloric acid, sodium dihydrogen phosphite and/or phosphate, and lesser amounts of reducing agent such as sodium hypophosphite, as well as the dissolved nickel salt. If another water-soluble nickel salt such as nickel sulfate is used, the corresponding acid is formed as the nickel is depleted. When caustic soda is added to such a bath to adjust its pH, and a water-soluble nickel salt such as nickel chloride is added to replenish the nickel content, there occurs an interreaction of the sodium hydroxide and nickel chloride and/or the hydrochloric acid already present to form sodium chloride or other undesirable by-products which accumulate and necessitate disposal of the plating solution.

I have now discovered that the above-mentioned difficulties can be avoided and the operating life of a chemical reduction plating bath can be greatly extended by utilizing a water-insoluble nickel salt as a source of nickel. More particularly, the water-insoluble nickel salts contemplated in the present invention are those adapted, when

2

dissolved in the plating solution, to regulate the bath pH, thus eliminating the necessity of separate additions of alkali.

Examples of suitable water-insoluble nickel salts are: 5 nickel oxy salts such as nickel monoxide, nickel peroxide, nickel sesquioxide, nickelous nickelic oxide, and nickel superoxide; hydroxy nickel salts such as nickelic hydroxide and nickelous hydroxide; and carbonates such as nickel carbonate and basic nickel carbonate. By employing one or more of these water-insoluble nickel salts as a source of nickel, either in replenishing a conventional chemical reduction bath or in the original bath makeup, not only is the desired nickel content provided, but also the bath pH is regulated by the alkaline radical liberated in the plating solution.

Typical of a nickel reduction plating bath which may be regulated in operation by the practice of the present invention is the following composition where the quantities expressed are per liter of water:

|    |                      |             |    |
|----|----------------------|-------------|----|
| 20 | Nickel chloride      | grams       | 30 |
|    | Sodium hypophosphite | do          | 10 |
|    | Glycollic acid (70%) | milliliters | 35 |
|    | Sodium hydroxide     | grams       | 15 |

25 It will be understood of course that the above bath composition is intended only as an illustration of a typical reduction plating bath and that the present invention is applicable to a wide range of bath compositions. For example, plating baths containing about 5 to 50 grams per liter of a water-soluble nickel salt such as nickel chloride, nickel acetate, nickel sulfate, etc.; approximately 5 to 100 grams per liter of a reducing agent, such as hypophosphorous acid, sodium hypophosphite or other soluble hypophosphites; and about 15 to 100 grams per liter of a buffer such as glycollic acid, sodium hydroxyacetate, sodium acetate, sodium citrate, etc. and/or other bath additives can similarly be replenished in accordance with the present invention.

30 Although various chemical reactions occur during the plating process and the bath replenishment, the exact interdependence of which is not clearly understood at present, the following reactions illustrate generally how the nickel salts of the present invention serve to replenish the nickel content and regulate the bath pH.

35 45 Employing nickel hydroxide:



Using basic nickel carbonate:



50 As shown in these reactions, when a nickel salt of the type contemplated in the present invention is added to the plating bath, a soluble nickel salt, namely, nickel chloride, is formed therein to replenish the nickel available for plating. Simultaneously, the hydrochloric acid which had been accumulating in the bath is neutralized to regulate the pH.

55 By employing water-insoluble nickel salts, the necessity of making frequent bath analyses for nickel content is eliminated. Moreover, the plating solution is not contaminated with by-product sodium chloride or other compounds, and since no foreign alkali need be added to the bath to regulate its pH, accurate pH determinations are no longer necessary.

60 While the present invention has thus far been described in some detail as being applicable for the replenishment and pH control of conventional reduction plating baths, it is to be understood that the present invention also contemplates the formation of an improved chemical reduction plating bath utilizing a water-insoluble nickel salt as

an initial ingredient. Such a bath comprises an aqueous mixture of a reducing agent and a water-insoluble nickel salt selected from the group consisting of oxy nickel salts, hydroxy nickel salts and nickel carbonates. In most instances it is desirable to additionally employ a buffer agent. A preferred bath of this type comprises nickel carbonate, sodium hypophosphite, and glycollic acid.

A bath of the above-mentioned type can be produced by dissolving the desired water-insoluble nickel salt or salts in glycollic acid and thereafter adding the reducing agent. If another type buffer is used, for example, sodium acetate, sodium citrate or sodium hydroxy acetate, the nickel salt may first be dissolved in hypophosphorus or phosphorus acid, enough acid being used to obtain the desired initial bath pH.

The following is an example of one reduction plating bath utilizing a water-insoluble nickel salt as an initial ingredient. The quantities expressed are per liter of water.

|                      |             |     |
|----------------------|-------------|-----|
| Nickel carbonate     | grams       | 15  |
| Glycollic acid (70%) | milliliters | 35  |
| Sodium hypophosphite | grams       | 10  |
| Preferred pH         |             | 5.0 |

A satisfactory range of ingredients comprises a mixture of about 5 to 100 grams per liter of a water-insoluble nickel salt, approximately 15 to 100 g. per liter of a buffer such as glycollic acid, sodium hydroxy acetate, sodium acetate, sodium citrate, etc., and about 5 to 100 grams per liter of reducing agent such as sodium hypophosphite, hypophosphorous acid, or other hypophosphites.

Since the nickel salts of the present invention are extremely insoluble in water, even at elevated temperatures, the use of these salts in the replenishment of conventional reduction nickel plating baths involves certain difficulties which I have succeeded in overcoming by the following method: A water-insoluble nickel salt is employed in the form of a slurry by stirring the finely divided nickel salt into water. The filter conventionally employed in chemical reduction plating systems is then coated with the finely divided water-insoluble nickel salt as by introducing the slurry into the filter intake. The used plating solution is then passed through the same filter whereby a quantity of the insoluble nickel salt is dissolved into the plating bath. In practice, the amount dissolved from the filter media will be approximately equivalent to the amount of nickel consumed in the plating. Hence, the plating bath will constantly replenish itself until the charge of the insoluble nickel salt has been consumed. Moreover, since the amount of nickel consumed in the reduction plating operation corresponds to the amount of acid produced, the alkaline radical liberated in solution by the gradual dissolving of the nickel salt will neutralize an equivalent amount of acid. Thus the pH will remain relatively constant.

In general, electroless nickel reduction plating baths of the type contemplated herein operate most satisfactorily at a pH within the range from about 3.5 to a pH at which nickel hydroxide is precipitated. A preferred pH range is from 5.0 to 5.5.

Plating baths embodying the present invention generally should be operated at a relatively high temperature for optimum results. I have found that the bath temperature in most instances should be at least 160° F. although a temperature within the range from about 190° F.-210° F. is preferred.

From the foregoing description it will now be understood that I have provided a new and different type chemical reduction nickel plating operation in which the nickel salt is replenished and the pH regulated by adding to the bath at periodic intervals, or continuously in certain applications, a water-insoluble nickel salt selected from the group consisting of nickel oxide, nickel hydroxide, nickel carbonate, and basic nickel carbonate. Also, in accordance with the invention, an additive to replenish or form

the bath consisting of a mixture of insoluble nickel compound, a hypophosphite reducing agent and buffer, if desired, may be used. The practice of the present invention provides convenient means for prolonging the operating life of a conventional type electroless nickel plating solution. Moreover, the invention also provides an improved plating solution in which an undesirable foreign ion need not be introduced and in which the production of an undesirable by-product is eliminated.

It is to be understood that, although the invention has been described with specific reference to particular embodiments thereof, it is not to be so limited since changes and alterations therein may be made which are within the full intended scope of this invention as defined by the appended claims.

What is claimed is:

1. In a chemical reduction plating process utilizing a plating bath comprising an aqueous solution of a water-soluble nickel salt and a hypophosphite reducing agent, the improvement which consists in maintaining the desired nickel concentration in the bath by additions of a water-insoluble nickel compound which is adapted to increase the pH of the plating bath.
2. In a chemical reduction nickel plating process of the type utilizing a plating bath comprising an aqueous solution of a water-soluble nickel salt and a soluble hypophosphite reducing agent, the improvement which consists of adding to the bath at least one water-insoluble nickel compound selected from the group consisting of nickel oxide, nickel hydroxide, nickel carbonate and basic nickel carbonate.
3. A method of maintaining the pH and desired nickel concentration in a chemical reduction nickel plating bath containing a soluble nickel salt and a soluble hypophosphite reducing agent, said method comprising the steps of preparing a water slurry of a water-insoluble nickel compound, depositing a coating of said slurry on a filter, and thereafter passing said nickel plating bath through said filter to dissolve therefrom an amount of water-insoluble nickel compound equivalent to the nickel consumed in plating.
4. In a chemical reduction nickel plating process of the type utilizing an aqueous plating solution comprising about 5 to 50 grams per liter of a water-soluble nickel salt, approximately 5 to 100 grams per liter of a hypophosphite reducing agent, and about 15 to 100 grams per liter of a buffer, the improvement which consists of replenishing the nickel content of said plating solution as it is depleted during plating by addition of at least one water-insoluble nickel compound selected from the group consisting of nickel oxide, nickel hydroxide, nickel carbonate, and basic nickel carbonate.
5. A chemical reduction type nickel plating bath comprising an aqueous solution of a nickel salt, a hypophosphite reducing agent and a buffer, said solution being in contact with a water-insoluble nickel compound so that acid generated in said bath during plating will react therewith to increase the pH and replenish the soluble nickel salt.
6. A chemical reduction type nickel plating bath comprising an aqueous solution of a soluble nickel salt, a hypophosphite reducing agent and a buffer, said solution being in contact with a nickel compound selected from the group consisting of nickel oxide, nickel hydroxide, nickel carbonate and the basic nickel carbonate.
7. In a chemical reduction nickel plating process of the type utilizing a plating bath comprising an aqueous solution of a water soluble nickel salt, a reducing agent selected from the group consisting of sodium hypophosphite and potassium hypophosphite, and a buffer, said bath being maintained at a pH of about from 3.5 to 6.0 and at a temperature of at least 160° F., the improvement which consists of regulating the pH and the desired nickel content of the bath during operation thereof by the addition of a nickel compound selected from the group consisting

of nickel oxide, nickel hydroxide, nickel carbonate, and basic nickel carbonate.

2,658,842 Gutzeit et al. Nov. 10, 1953  
2,726,969 Spaulding Dec. 13, 1955

## References Cited in the file of this patent

## UNITED STATES PATENTS

1,003,092 Dow et al. Sept. 12, 1911  
2,541,721 Roehl et al. Feb. 13, 1951  
2,658,839 Talmey et al. Nov. 10, 1953  
2,658,841 Gutzeit et al. Nov. 10, 1953 10

5 Blum et al.: Principles of Electroplating and Electro-forming, 3rd edition, 1949, pages 363-364.  
Hodgman et al.: "Handbook of Chemistry and Physics," Chemical Rubber Publishing Co., Cleveland, 26th ed. (1942), p. 416.

## OTHER REFERENCES